

Dec. 23, 1958

J. A. NEWTON ET AL

2,865,359

POPPET VALVE WITH WEAR RESISTANT STEM TIP

Filed May 18, 1955



FIG. 2



FIG. 3



INVENTORS  
JOHN A. NEWTON  
MAX J. TAUSCHEK

By *John Sherman, Mamo, Clegg, Simpson* Atty's.

# United States Patent Office

2,865,359

Patented Dec. 23, 1958

1

2,865,359

## POPPET VALVE WITH WEAR RESISTANT STEM TIP

John A. Newton, Painesville, and Max J. Tauschek, Lyndhurst, Ohio, assignors to Thompson Products, Inc., Cleveland, Ohio, a corporation of Ohio

Application May 18, 1955, Serial No. 509,312

2 Claims. (Cl. 123—188)

This invention relates to a valve with a tipped stem and method of forming the same and more particularly to a valve having the impact end of its stem recessed and provided with an impact nubbin fused to the stem in the recess.

In the manufacture of automobile valves of alloy metal it has been the practice to provide the impact end of the valve stem with a tip or nubbin of harder metal than that of the stem so as to increase the wearing ability or longevity of the valve in use.

Heretofore, the tip or nubbin has been simply welded on the flat surface at the end of the stem. This practice has been especially followed in the manufacture of aircraft valves. It has been found, however, that such welded tips resulted in a high rate of manufactured rejects due to cracks and inadequate bonding of the tip to the stem.

An object, therefore, of this invention is to provide an improved impact tip for a valve stem which lends itself to economical manufacture on a large production scale.

Still another object of the invention is to provide a simple but inexpensive method of more effectively fusing a tip or nubbin to the valve stem so that such tip is actually embodied as an end insert substantially within the confines of the length of the stem.

Yet another object of this invention is to provide a valve stem impact tip of improved metallic composition which will better stand up at the wear point of the end of the stem.

In accordance with the general features of this invention, there is provided an article of manufacture comprising a valve having a valve stem provided at its impact end with a dished recess and an insert nubbin in the recess of a metal alloy of harder characteristic than that of the stem bonded to the stem so as to be integral therewith.

In accordance with other features of the invention, there is provided in a method of forming the impact end of a metallic valve stem with an impact tip of harder metal than that of the stem, the steps of providing the valve end with a dished recess, puddling a molten metal alloy of harder characteristic than that of the stem in the recess and fusing the puddled metal to the stem to provide it with an integral tip.

Another feature of the invention relates to the striating or laminating of the valve stem tip or insert.

Other objects and features of the invention will more fully appear from the following detailed description taken in connection with the accompanying drawings which illustrate several embodiments thereof, and in which:

Figure 1 is a fragmentary view of a rocker arm and valve assembly with a valve embodying this invention;

Figure 2 is a fragmentary vertical sectional view through a valve stem having a tip with the features of this invention; and

Figure 3 is a view similar to Fig. 2 showing a striated or laminated insert.

2

As shown on the drawings:

It is believed that this invention will be best understood by first describing a valve assembly of the type used in automobile and aircraft engines to which the valve made pursuant to the present method can be used. In Fig. 1, it will be perceived that a conventional rocker arm is designated by the reference numeral 10 and is shown in coaction with a valve 11. The rocker arm and valve assembly may be of any suitable conventional construction in which motion is imparted to the valve by an impact force exerted against the end of the valve stem 12. As is known such motion, in the cycle of an engine, is imparted to the valve by the rocker arm 10 for unseating or opening the valve 11.

The valve 11 may be made of any suitable metal, although excellent results may be obtained in engines such as aircraft engines by making the valve of an austenitic nickel base alloy. Desirable results may be attained by the use of an alloy of the following composition:

|           |            |
|-----------|------------|
| Chromium  | 15-17.     |
| Titanium  | 2.75-3.35. |
| Manganese | 2. to 2.5. |
| Iron      | 8 max.     |
| Carbon    | .07 max.   |
| Silicon   | .15 max.   |
| Sulphur   | .01 max.   |
| Aluminum  | .1 max.    |
| Copper    | .2 max.    |
| Nickel    | Balance.   |

In accordance with the features of this invention, the valve stem 12 has its tip or impact end provided with a dished or arcuate recess 13 with maximum depth at the axis of the stem and minimum depth at the periphery of the stem. Disposed in this recess and bonded to the stem is an alloy metal insert, disk or nubbin 14 preferably applied pursuant to the instant method to be hereinafter described.

This insert is made of a harder alloy metal than that of the stem proper. Excellent results may be attained for aircraft purposes by using an alloy in this insert of the following order:

|                         |            |
|-------------------------|------------|
| Chromium                | 28.0-32.0. |
| Tungsten                | 11.0-14.0. |
| Carbon                  | 2.60-3.0.  |
| Nickel                  | 3.0 max.   |
| Iron                    | 3.0 max.   |
| Silicon                 | 1.5 max.   |
| Manganese               | 1.0 max.   |
| Molybdenum              | 1.0 max.   |
| Other impurities, total | 1.0 max.   |
| Cobalt                  | Remainder. |

The metal for the insert may be obtained in the form of cast rod, preferably with surface fins and projections removed by grinding. The material of the rod should demonstrate good weldability and shall flow smoothly and evenly under inert gas shielded arc or oxy-acetylene welding without bubbling or boiling so as to produce an adherent deposit free from porosity, and when molten, shall have sufficient surface tension to permit ease of build-up of the deposit.

In addition, the material after being welded or fused as contemplated and after grinding should have a hardness of 50 to 55 on a Rockwell "C" scale.

In the formation of the insert 14 in the stem 12 from the alloy rod stock (not shown), any suitable inert gas shielded arc or oxy-acetylene welding equipment may be used. It will be appreciated that the stem is disposed with its recessed end uppermost. Then the alloy metal rod is disposed in the recess 13 and is rendered molten

by welding and progressively puddled in the recess until the desired depth of insert 14 is provided. It has been found that the insert should be of the order of  $\frac{1}{8}$  inch at the wear or impact point to preclude deleterious dilution of the stem metal into the alloy such as would soften the alloy. In this manner, the metal is puddled in and fused to the end of the stem.

Thereafter any suitable equipment may be employed for flat grinding the exposed surface of the insert or nubbin 14. It will be observed that this insert or nubbin 10 14 is bodily disposed substantially within the confines of the length of the stem. This is to be distinguished from previous practices of merely butt welding a tip on a stem.

As an alternative, the metal of the insert may be puddled and bonded in striated or laminated form as indicated at 14' in Fig. 3. This modified form of insert 14' is composed of a series of layers of laminations 15' superimposed one upon the other in the recess 13' at the end of the valve stem 12'. By virtue of the laminations in the modification the outer successively puddled and welded laminations would not be affected by dilution of valve stem metal since they are bonded to the metal of the initial or first lamination.

In both forms the insert 14—14' by virtue of its alloy and the fact that it has a Rockwell "C" hardness of the 25 order of 50 will reduce to a negligible minimum manufacturing rejects as compared to rejects of as much as 50% in previous practices. In addition, not only is a better and stronger bonding of the insert made possible by virtue of it being puddled in the recess, but in addition a very augmented wearing area or point is provided at the impact locale of the stem end.

We claim as our invention:

1. An internal combustion engine poppet valve having a metal stem with stem metal closing the end of the stem and forming a solid dished impact end providing a recess within the circumference of the stem, a high carbon cobalt base alloy insert nubbin of harder characteristic than the stem metal integrally united to the stem throughout the entire area of said dished end, said dished end having a 40 bottom of arcuate contour with a substantially deep maxi-

5 mum depth along the axis of the stem and with a minimum depth adjacent the circumference of the stem, and said insert nubbin being a solidified puddle with a junction bond along the entire extent of said arcuate bottom and having a substantially flat outer face forming a wear-resisting impact surface, the wear-resistant surface of said nubbin being substantially undiluted with stem metal, and the bond between the nubbin and dished end of the stem extending into both the nubbin and stem metals.

2. An internal combustion engine poppet valve especially adapted for aircraft engines which comprises a valve body having a stem with stem metal forming a closed solid stem end, the solid end of said stem having a deeply dished recess in the end face thereof with a maximum depth at the axis of the valve stem and a minimum depth adjacent the circumference of the valve stem, a solidified puddle of high carbon cobalt base alloy bodily disposed within the confines of the length of the stem in said recess in integral relation with the stem metal throughout a bond area extending substantially into both the stem metal and the puddle metal along the entire contour of the recess, said nubbin having a substantially flat outer impact face adapted to resist wear, and the metal constituting said face being substantially undiluted by stem metal.

#### References Cited in the file of this patent

#### UNITED STATES PATENTS

|           |                 |                |
|-----------|-----------------|----------------|
| 1,526,385 | Smith           | Feb. 17, 1925  |
| 1,628,911 | Rich            | May 17, 1927   |
| 1,699,273 | Bissell         | Jan. 15, 1929  |
| 1,823,452 | Heron           | Sept. 15, 1931 |
| 1,823,454 | Jardine         | Sept. 15, 1931 |
| 1,889,916 | Colwell         | Dec. 6, 1932   |
| 1,904,430 | Ferrando et al. | Apr. 18, 1933  |
| 2,089,749 | Jardine         | Aug. 10, 1937  |
| 2,280,758 | Voorhies        | Apr. 21, 1942  |
| 2,407,561 | Lincoln         | Sept. 10, 1946 |

#### FOREIGN PATENTS

|         |               |               |
|---------|---------------|---------------|
| 431,547 | Great Britain | July 10, 1935 |
|---------|---------------|---------------|